

2,982,702

## PRETREATING URANIUM FOR METAL PLATING 5

Ralph F. Wehrmann, Waukegan, Ill., assignor to the United States of America as represented by the United States Atomic Energy Commission

No Drawing. Filed May 9, 1950, Ser. No. 161,020

2 Claims. (Cl. 204—1.5)

This invention deals with a process for pretreating uranium prior to applying metal coatings and the compositions suitable therefor.

Uranium is a highly reactive metal and oxidizes when in contact with air. The oxide films formed thereby are very disadvantageous when the uranium article is to be metal-coated because they are responsible for a very poor adherence of the metal coating to the uranium surface.

It is an object of this invention to provide a process for treating uranium metal to remove oxide surface layers therefrom.

It is another object of this invention to provide a process for treating uranium articles by which a very smooth surface is obtained.

It is another object of this invention to provide a process for treating uranium by which its surface is preconditioned so that a metal coating then applied is firmly bonded thereto.

It is thus also an object of this invention to provide a process for preparing uranium articles for metal plating.

Still another object of this invention is to provide a process for treating uranium whereby its surface is uniformly attacked without the occurrence of pitting.

It is finally still another object of this invention to provide a process for treating uranium surfaces by which very little metal is removed.

These and other objects are accomplished by contacting the surface of the uranium articles with an aqueous mixture of polycarboxylic acid and hydrochloric acid. The concentrations of the acids can be varied widely.

The process of this invention can be carried out by simply immersing the article into the solution or else the article may be given an anodic treatment. While all kinds of polycarboxylic acids which are water-soluble, including oxalic, citric, malonic, tartaric, malic and glutaric acids, are suitable for the process of this invention, oxalic acid is preferred.

The results of the process of this invention can still be further improved by adding glycerine to the carboxylic acid-hydrochloric acid aqueous mixture. Proportions of from 1 to 5% by weight of each, hydrochloric acid and glycerine are the optimal ranges. A concentration of 10% with regard to the oxalic acid has given excellent results. Glycerine and hydrochloric acid can be added to the oxalic acid solution in about equal amounts; however, this is not obligatory.

The process can be carried out at room temperature, i.e., at a temperature between 20° and 35° C., or the solution can be heated to a temperature below its boiling point. The time of immersion, of course, is dependent upon the thickness of the oxide layer to be removed. In general, immersion times of from thirty seconds to fifteen minutes have been found suitable.

When the treatment is carried out anodically, a current density of from 60–100 amperes/ft.<sup>2</sup> gives excellent results. In this case, the temperature preferably ranges from 40° to 75° C.

It is advantageous, though optional, mechanically to clean the uranium metal surface prior to the treatment by the process of this invention. This may be carried out by immersing the metal into a degreasing agent, such as trichloroethylene, and/or sandblasting the surface. For instance, sandblasting with 120 mesh steel grit for two to three minutes has been found satisfactory.

After the treatment with the oxalic acid-hydrochloric acid mixture, with or without the glycerine, the article is preferably rinsed by, or immersed into, a nitric acid solution; nitric acid obtained by diluting concentrated nitric acid with an equal amount of water and an immersion time of from one to ten minutes were found satisfactory for this purpose. Instead of, or in addition to, the nitric acid, the article may also be rinsed with water either of room temperature or of elevated temperature.

In the following, an example is given of the process of this invention.

20 Uranium metal was immersed in a 10% aqueous solution of oxalic acid which contained 20 cc./liter each of glycerine and concentrated hydrochloric acid. The solution had a temperature of 40° C., and the article was immersed for thirty minutes. Thereafter, the thus treated article was immersed into nitric acid obtained by mixing commercial concentrated nitric acid with an equal volume of water for approximately ten minutes and rinsed with water. The thus pretreated article was then given a copper coating of a thickness of 1 mil by a conventional electrolytical method. The coating showed excellent adherence and had a very bright surface. The coated uranium article is suitable for use in a neutronic reactor of the type described in the copending application of Fermi et al., Serial No. 568,904, filed December 19, 1944, 25 granted as U.S. Patent No. 2,708,656 on May 17, 1955.

30 It will be understood that this invention is not to be limited to the details given herein but that it may be modified within the scope of the appended claims. The invention, for instance, is not only applicable to preparing uranium for plating with copper but also for plating with other metals. Likewise, the process of this invention has utility as a pretreatment for various methods of plating, whether, for instance, carried out by immersion or electrolytically.

35 40 45 What is claimed is:

1. A process for pretreating uranium for metal plating, comprising anodically treating a uranium article at a current density of from 60 to 100 amperes/ft.<sup>2</sup> in an aqueous solution of about 10% polycarboxylic acid, from 1 to 5% by weight of glycerine and from 1 to 5% by weight of hydrochloric acid for from 30 seconds to 15 minutes, said solution having a temperature of from 20° to 75° C.

50 55 2. The process of claim 1 wherein the polycarboxylic acid is oxalic acid.

## References Cited in the file of this patent

## UNITED STATES PATENTS

|    |           |                |               |
|----|-----------|----------------|---------------|
| 60 | 31,880    | Ely            | Apr. 2, 1861  |
|    | 1,011,203 | Jahn           | Dec. 12, 1911 |
|    | 1,462,421 | Pearson et al. | July 17, 1923 |
|    | 1,495,538 | Thews          | May 27, 1924  |
|    | 1,526,943 | Thews          | Feb. 17, 1925 |
| 65 | 1,757,959 | Gravel         | May 13, 1930  |
|    | 1,994,633 | Boyd           | Mar. 19, 1935 |
|    | 2,287,050 | Miller         | June 23, 1942 |
|    | 2,318,559 | Percival       | May 4, 1943   |
|    | 2,465,987 | Gorman         | Apr. 5, 1949  |

## FOREIGN PATENTS

|    |        |               |      |
|----|--------|---------------|------|
| 70 | 16,548 | Great Britain | 1902 |
|    | 139    | Great Britain | 1911 |